# EUROPEAN PATENT SPECIFICATION

(11) **EP 2 449 140 B1**
(45) Date of publication and mention of the grant of the patent: **20.05.2015**
(21) Application number: 10727610.7
(22) Date of filing: 15.06.2010
(51) Int. Cl.: C22C 1/02, C22C 19/05, F01D 5/06, F01D 9/02

(54) **NICKEL BASE SUPERALLOY COMPOSITIONS AND ARTICLES THEREOF**
ZUSAMMENSETZUNGEN VON SUPERLEGIERUNGEN AUF BASIS VON NICKEL UND BAUTEILE DARAUS
COMPOSITIONS DE SUPERALLIAGES À BASE DE NICKEL ET COMPOSANT EN CES COMPOSITIONS

(30) Priority: 04.06.2010 US 794244; 30.06.2009 US 221946 P
(43) Date of publication of application: 09.05.2012
(73) Proprietor: General Electric Company, Schenectady, NY 12345 (US)
(72) Inventor: MILLER, Joshua, Leigh, Cincinnati, OH 45215 (US); HAZEL, Brian, Thomas, Cincinnati, OH 45215 (US); KONITZER, Douglas, Gerard, Cincinnati, OH 45215 (US); FINK, Paul, John, Cincinnati, OH 45215 (US)
(74) Representative: Szary, Anne Catherine
(86) International application number: PCT/US2010/038640
(87) International publication number: WO 2011/002605

(56) References cited:
- WO-A1-2009/032578
- WO-A1-2009/032579
- WO-A1-2009/085420

## Description

This invention relates generally to nickel-base superalloy compositions and superalloy articles and more particularly to such alloys for use in high pressure turbine (HPT) nozzle applications.

Currently known no-rhenium superalloys may exhibit inadequate stress rupture capability. Other known superalloys that provide desired stress rupture capability may include relatively high amounts of rhenium. It is desirable to provide an alloy able to provide sufficient stress rupture capability with a reduced rhenium level.

WO 2009/032579 discloses a nickel base superalloy composition substantially free of rhenium includes, in percentages by weight: about 5-8 Cr; about 7-8 Co; about 1.3-2.2 MO; about 4.75-6.75 W; about 6.0-7.0 Ta; if present, up to about 0.5 Ti; about 6.0-6.4 Al; about 0.15-0.6 Hf; if present, from about 0.03-0.006 C; if present, up to about 0.004 B; if present, one or more rare earths selected from Y, La and Ce up to about 0.03 total, the balance including nickel and incidental impurities. The superalloy composition is able to provides sustained-peak low cycle fatigue and/or oxidation resistance properties comparable to second generation superalloy compositions including at least about 3 wt% rhenium. Superalloy articles incorporating the compositions include nozzles, shrouds, and splash plates for gas turbine engines.

WO 2009/085420 discloses a stabilized superalloy composition comprises tungsten, molybdenum, and optionally rhenium, the superalloy composition being modified with a stabilizing amount of hafnium sufficient to decrease the formation of topologically close packed (TCP) phases in a superalloy microstructure at elevated temperatures with respect to a comparable unmodified superalloy composition. Articles exhibiting increased microstructure stability formed from hafnium-modified superalloy compositions may be utilized in gas turbine engines. Methods for stabilizing superalloy compositions at elevated temperatures include utilizing hafnium as a stabilizer to decrease the propensity to form TCP phases.

### SUMMARY OF THE INVENTION

The above-mentioned need or needs may be met by the alloy as defined in the claims that provides nickel-base superalloy compositions for use in high temperature applications. Exemplary embodiments exhibit sufficient stress rupture capability, at relatively low- or no- rhenium levels.

The superalloy composition consists of, in weight percent: 6.2-6.6 aluminum (Al), 6.5-7.0 tantalum (Ta), 6.0 chromium (Cr), 6.25-7.0 tungsten (W), 2.0 molybdenum (Mo), 0.60 hafnium (Hf), 0.5 rhenium (Re), 7.5 cobalt (Co), optionally, 0.03-0.06 carbon (C), optionally, up to 0.004 boron (B,) optionally up to 0.03 total of one or more rare earth elements selected from yttrium (Y), lanthanum (La), or cerium (Ce), balance nickel (Ni). The superalloy composition exhibits a stress rupture capability improvement of at least about 15% over a base stress rupture capability of a base composition nominally comprising, in weight percent: 6.5 Al, 6.6 Ta, 6.0 Cr, 6.25 W, 1.5 Mo, 0.15 Hf, 0.0 Re, 7.5 Co, balance nickel.

In an exemplary embodiment, a superalloy composition consists of, in weight percent: 6.3 aluminum (Al), 6.5 tantalum (Ta), 6.0 chromium (Cr), 6.25-7.0 tungsten (W), 2.0 molybdenum (Mo), 0.6 hafnium (Hf), 0.0 rhenium (Re), 7.5 cobalt (Co), optionally, 0.03-0.06 carbon (C), optionally, up to 0.004 boron (B), optionally up to 0.03 total of one or more rare earth elements selected from yttrium (Y), lanthanum (La), or cerium (Ce), and a balance of nickel (Ni) and incidental impurities.

In an exemplary embodiment, an article formed from an exemplary superalloy composition is provided. The article may be a high pressure turbine nozzle, nozzle segment, or other gas turbine engine component.

### BRIEF DESCRIPTION OF THE DRAWINGS

The subject matter which is regarded as the invention is particularly pointed out and distinctly claimed in the concluding part of the specification. The invention, however, may be best understood by reference to the following description taken in conjunction with the accompanying drawing figures in which:
FIG. 1 is a perspective view of a component article such as a gas turbine engine high pressure turbine (HPT) nozzle segment.

### DETAILED DESCRIPTION OF THE INVENTION

Referring now to the drawings, FIG. 1 depicts an HPT nozzle segment 10 including at least one vane 12. In an exemplary embodiment, the nozzle segment 10 comprises a single crystal nickel-base superalloy composition as disclosed herein. Articles incorporating the disclosed superalloy composition include HPT nozzles or nozzle segments and may include other gas turbine engine components.

Exemplary nickel-base superalloy composition comprise reduced levels of rhenium (Re), defined herein as being from 0 up to 0.5 weight %. Increased amounts of other strengthening alloying elements such as tantalum (Ta), tungsten (W) and molybdenum (Mo) may be utilized to offset the lower levels of Re. Tantalum may be present in amounts from 6.5 to 7.0 weight %, molybdenum may be present in amounts of 2.0 weight %, and tungsten may be present in amounts from 6.25 to 7.0 weight %. In other exemplary embodiments, tantalum may be present at levels of from 6.5 to 6.6 weight %. All percentages presented herein are percentages by weight, unless noted otherwise.

Table 1 provides a series of exemplary compositions. A theoretical stress rupture prediction generated by computer modeling for the compositions was compared with the predicted stress rupture (in hours) of a base, no-rhenium superalloy composition. As evidenced in Table 1, each of the enumerated compositions provided an improved predicted stress rupture, presented as % improvement.

Certain of the exemplary compositions presented in Table 1 are highlighted. These exemplary compositions exhibit excellent improvement in the predicted stress rupture as compared to the Base composition. These exemplary compositions may provide desired outcomes with reduced rhenium levels (0.0-0.5 weight %).

Alloys 25 and 27 listed in Table 1 are provided as comparative examples and include about 1.5 weight % rhenium. Exemplary embodiments disclosed herein consider the contributions of various alloying elements to the thermal mechanical properties and oxidation resistance of the superalloy composition.

The alloy contains from 6.2 to 6.6 weight percent aluminum. In other exemplary embodiments, the aluminum may be present in amounts from 6.3 to 6.5 percent.

The alloy contains 6 weight % chromium (Cr) to sufficient to provide hot corrosion resistance, but not high enough to detrimentally lead to TCP chase instability and poor cyclic oxidation resistance.

The alloy contains 7.5% cobalt (Co). Lower amounts of cobalt may reduce alloy stability. Greater amounts may reduce the gamma prime solvus temperature thus impacting high temperature strength and oxidation resistance.

The alloy contains molybdenum (Mo) in an amount of 2.0 weight %. Greater amounts of Mo may also negatively impact both hot corrosion and oxidation resistance.

The alloy contains tungsten (W) in an amount from 6.25 to 7.0 weight %. Lower amounts of W may decrease strength. Higher amounts may produce instability with respect to TCP phase formation. Higher amounts may also reduce oxidation capability.

The alloy contains reduced levels of rhenium, from 0.0 to 0.5 weight percent. It is contemplated that some or all of the rhenium may be provided as revert from scrap material. It is desired to provide improved performance at reduced rhenium levels.

Hafnium (Hf) is included at 0.6 weight %. Hafnium can improve oxidation resistance and the adherence of thermal barrier coatings when utilized. However, hafnium can degrade the corrosion resistance of uncoated alloys. Hafnium additions of greater than about 1% adversely impact stress rupture properties and the incipient melting temperature.

Optional additions may include 0.03-0.06 weight % carbon (C), up to 0.004 weight % boron (B), or up to 0.03 weight% of one or more rare earth elements such as yttrium (Y), lanthanum (La), and cesium (Ce).

Boron provides strength for low angle boundaries and enhanced acceptability limits for components having low angle grain boundaries. The lower limit for carbon provides sufficient carbon to improve alloy cleanliness since carbon provides de-oxidation. Beyond the upper 0.06% amount, the carbide volume fraction increases, reducing fatigue life. Rare earth additions, i.e., yttrium (Y), lanthanum (La), and cerium (Ce), may be provided in certain embodiments in amounts up to 0.03%. These additions may improve oxidation resistance by enhancing the retention of the protective alumina scale. Greater amounts may promote mold/metal reaction at the casting surface, increasing the component inclusion content.

Exemplary embodiments disclosed herein include each of the enumerated compositions in Table 1 with the exception of the base composition, and comparative alloys 25 and 27. Additionally, exemplary embodiments disclosed herein include compositions employing the endpoints of disclosed ranges and all intermediate values. For example, a range of aluminum from 6.2 to 6.6 weight percent is defined to include 6.2 weight percent, 6.6 weight percent, and any intervening percentage between 6.2 and 6.6 weight percent.

Exemplary embodiments disclosed herein provide improved stress rupture capability of at least 15% as compared to a base stress rupture capability of a base composition nominally comprising, in weight percent: 6.5 Al, 6.6 Ta, 6.0 Cr, 6.25 W, 1.5 Mo, 0.15 Hf, 0.0 Re, 7.5Co, balance Ni, identified as "Base" in Table 1.

### EXAMPLES

**TABLE 1**

| **Alloy** | **Al** | **Ta** | **Cr** | **W** | **Mo** | **Hf** | **Re** | **Co** | **% Improved** |
|---|---|---|---|---|---|---|---|---|---|
| Base | 6.5 | 6.6 | 6.0 | 6.25 | 1.5 | 0.15 | 0.0 | 7.5 | --- |
| 1 | 6.3 | 6.5 | 6.0 | 6.25 | 2.0 | 0.60 | 1.0 | 7.5 | 154 |
| 2 | 6.3 | 6.5 | 6.0 | 6.25 | 2.0 | 0.60 | 0.5 | 7.5 | 117 |
| 6 | 6.5 | 6.6 | 6.0 | 6.25 | 1.5 | 0.15 | 0.5 | 7.5 | 33 |
| 7 | 6.5 | 6.6 | 6.0 | 6.25 | 1.5 | 0.15 | 1.0 | 7.5 | 70 |
| 8 | 6.5 | 6.6 | 6.0 | 6.25 | 1.5 | 0.60 | 0.5 | 7.5 | 83 |
| 9 | 6.5 | 6.6 | 6.0 | 6.25 | 1.5 | 0.60 | 1.0 | 7.5 | 135 |
| 10 | 6.5 | 6.6 | 6.0 | 6.25 | 1.5 | 0.60 | 0.0 | 7.5 | 40 |
| 11 | 6.3 | 6.5 | 7.0 | 6.25 | 2.0 | 0.60 | 1.0 | 7.5 | 114 |
| 12 | 6.3 | 6.5 | 7.0 | 6.25 | 2.0 | 0.60 | 0.5 | 7.5 | 94 |
| 13 | 6.5 | 6.6 | 7.0 | 6.25 | 1.5 | 0.15 | 0:5 | 7.5 | 52 |
| 14 | 6.5 | 6.6 | 7.0 | 6.25 | 1.5 | 0.15 | 1.0 | 7.5 | 84 |
| 15 | 6.5 | 6.6 | 7.0 | 6.25 | 1.5 | 0.60 | 0.5 | 7.5 | 104 |
| 16 | 6.5 | 6.6 | 7.0 | 6.25 | 1.5 | 0.60 | 1.0 | 7.5 | 122 |
| 17 | 6.5 | 6.6 | 7.0 | 6.25 | 1.5 | 0.60 | 0.0 | 7.5 | 74 |
| 18 | 6.3 | 6.5 | 6.5 | 6.25 | 2.0 | 0.60 | 1.0 | 7.5 | 139 |
| 19 | 6.3 | 6.5 | 6.5 | 6.25 | 2.0 | 0.60 | 0.5 | 7.5 | 81 |
| 20 | 6.5 | 6.6 | 6.5 | 6.25 | 1.5 | 0.15 | 0.5 | 7.5 | 45 |
| 21 | 6.5 | 6.6 | 6.5 | 6.25 | 1.5 | 0.15 | 1.0 | 7.5 | 78 |
| 22 | 6.5 | 6.6 | 6.5 | 6.25 | 1.5 | 0.60 | 0.5 | 7.5 | 103 |
| 23 | 6.3 | 6.6 | 6.5 | 6.25 | 1.5 | 0.60 | 1.0 | 7.5 | 143 |
| 24 | 6.5 | 6.6 | 6.5 | 6.25 | 1.5 | 0.60 | 0.0 | 7.5 | 61 |
| *25 | 6.3 | 6.5 | 7.0 | 6.25 | 2.0 | 0.60 | 1.5 | 7.5 | 128 |
| 26 | 6.5 | 6.6 | 7.0 | 6.25 | 1.5 | 0.15 | 0.0 | 7.5 | 24 |
| *27 | 6.3 | 6.5 | 6.5 | 6.25 | 2.0 | 0.60 | 1.5 | 7.5 | 160 |
| 28 | 6.5 | 6.6 | 6.5 | 6.25 | 1.5 | 0.15 | 0.0 | 7.5 | 15 |
| 29 | 6.3 | 6.5 | 6.0 | 7.00 | 2.0 | 0.60 | 0.0 | 7.5 | 102 |
| 30 | 6.3 | 6.5 | 7.0 | 7.00 | 2.0 | 0.60 | 0.0 | 7.5 | 76 |
| 31 | 6.3 | 6.5 | 6.0 | 7.00 | 2.0 | 0.60 | 0.5 | 7.5 | 138 |
| 32 | 6.3 | 6.5 | 7.0 | 7.00 | 2.0 | 0.60 | 0.5 | 7.5 | 92 |
| 33 | 6.3 | 6.5 | 6.0 | 7.00 | 2.5 | 0.60 | 0.0 | 7.5 | 87 |
| 34 | 6.3 | 6.5 | 7.0 | 7.00 | 2.5 | 0.60 | 0.0 | 7.5 | 51 |
| 35 | 6.3 | 6.5 | 6.0 | 7.00 | 2.5 | 0.60 | 0.5 | 7.5 | 122 |
| 36 | 6.3 | 6.5 | 7.0 | 7.00 | 2.5 | 0.60 | 0.5 | 7.5 | 83 |
| 37 | 6.3 | 6.5 | 6.0 | 6.50 | 2.0 | 0.60 | 0.0 | 7.5 | 87 |
| 38 | 6.3 | 6.5 | 7.0 | 6.25 | 2.0 | 0.60 | 0.0 | 7.5 | 71 |
| 39 | 6.3 | 6.5 | 6.0 | 6.50 | 2.0 | 0.60 | 0.5 | 7.5 | 124 |
| 40 | 6.3 | 6.5 | 7.0 | 6.50 | 2.0 | 0.60 | 0.5 | 7.5 | 94 |
| 41 | 6.3 | 6.5 | 6.0 | 6.50 | 2.5 | 0.60 | 0.0 | 7.5 | 78 |
| 42 | 6.3 | 6.5 | 7.0 | 6.50 | 2.5 | 0.60 | 0.0 | 7.5 | 46 |
| 43 | 6.3 | 6.5 | 6.0 | 6.50 | 2.5 | 0.60 | 0.5 | 7.5 | 115 |
| 44 | 6.3 | 6.5 | 7.0 | 6.50 | 2.5 | 0.60 | 0.5 | 7.5 | 77 |
| All: Balance Ni 25 and 27 include 1.5 weight % Rhenium as comparative | | | | | | | | | |

Examples 2, 29, 31, 37 and 39 illustrate the invention.

## Claims

1. A superalloy composition consisting of, in weight percent: 6.2-6.6 aluminum (Al), 6.5-7.0 tantalum (Ta), 6.0 chromium (Cr), 6.25-7.0 tungsten (W), 2.0 molybdenum (Mo), 0.6 hafnium (Hf), from 0.0 to 0.5 rhenium (Re), 7.5 cobalt (Co), optionally, 0.03-0.06 carbon (C), optionally, up to 0.004 boron (B), optionally up to 0.03 total of one or more rare earth elements selected from yttrium (Y), lanthanum (La), or cerium (Ce), and a balance of nickel (Ni) and incidental impurities.

2. The superalloy composition according to claim 1 consisting of 6.5 to 6.6 weight percent tantalum.

3. The superalloy composition according to claim 1 consisting of 0 weight percent rhenium.

4. The superalloy composition according to claim 1 consisting of 0.5 weight percent rhenium.

5. The superalloy composition according to claim 1, consisting of, in weight percent: 6.3 aluminum (Al), 6.5 tantalum (Ta), 6.0 chromium (Cr), from 6.25 to 7 tungsten (W), 2.0 molybdenum (Mo), 0.60 hafnium (Hf), 0.0 rhenium (Re), 7.5 cobalt (Co), optionally, 0.03-0.06 carbon (C), optionally, up to 0.004 boron (B), optionally up to 0.03 total of one or more rare earth elements selected from yttrium (Y), lanthanum (La), or cerium (Ce), and a balance of nickel and incidental impurities.

6. An article formed of a superalloy composition according to claim 1 or claim 5.

7. The article according to claim 6 comprising a gas turbine engine component.

8. The article according to claim 7 comprising a high pressure turbine nozzle or nozzle segment.

## Patentansprüche

1. Superlegierungs-Zusammensetzung, bestehend aus, in Gewichtsprozent: 6,2-6,6 Aluminium (Al), 6,5-7,0 Tantal (Ta), 6,0 Chrom (Cr), 6,25-7,0 Wolfram (W), 2,0 Molybden (Mo), 0,6 Hafnium (Hf), von 0,0 bis 0,5 Rhenium (Re), 7,5 Cobalt (Co), optional 0,03-0,06 Kohlenstoff (C), optional bis zu 0,004 Bor (B), optional bis zu 0,03 insgesamt aus einem oder mehreren Seltenerdelementen, ausgewählt aus Yttrium (Y), Lanthan (La) oder Cer (Ce) und einem Rest aus Nickel (Ni) und gelegentlichen Unreinheiten.

2. Superlegierungs-Zusammensetzung nach Anspruch 1, bestehend zu 6,5 bis 6,6 Gew.-% aus Tantal.

3. Superlegierungs-Zusammensetzung nach Anspruch 1, bestehend zu 0 Gew.-% aus Rhenium.

4. Superlegierungs-Zusammensetzung nach Anspruch 1, bestehend zu 0,5 Gew.-% aus Rhenium.

5. Superlegierungs-Zusammensetzung nach Anspruch 1, bestehend aus, in Gewichtsprozent: 6,3 Aluminium (Al), 6,5 Tantal (Ta), 6,0 Chrom (Cr), von 6,25 bis 7 Wolfram (W), 2,0 Molybden (Mo), 0,60 Hafnium (Hf), 0,0 Rhenium (Re), 7,5 Cobalt (Co), optional 0,03-0,06 Kohlenstoff (C), optional bis zu 0,004 Bor (B), optional bis zu 0,03 insgesamt aus einem oder mehreren Seltenerdelementen, ausgewählt aus Yttrium (Y), Lanthan (La) oder Cer (Ce) und einem Rest aus Nickel und gelegentlichen Unreinheiten.

6. Artikel aus einer Superlegierungs-Zusammensetzung nach Anspruch 1 oder Anspruch 5.

7. Artikel nach Anspruch 6, umfassend eine Gasturbinenmotor-Komponente.

8. Artikel nach Anspruch 7, umfassend einen Hochdruckturbinenleitkranz oder ein Leitkranzsegment.

## Revendications

1. Composition de superalliage constituée, en pourcentage en poids, des éléments suivants : 6,2 à 6,6 d'aluminium (Al), 6,5 à 7,0 de tantale (Ta), 6,0 de chrome (Cr), 6,25 à 7,0 de tungstène (W), 2,0 de molybdène (Mo), 0,6 d'hafnium (Hf), 0,0 à 0,5 de rhénium (Re), 7,5 de cobalt (Co), éventuellement, 0,03 à 0,6 de carbone (C), éventuellement, jusqu'à 0,004 de bore (B), éventuellement jusqu'à 0,03 au total d'un ou plusieurs éléments de terres rares choisis parmi l'yttrium (Y), le lanthane (La) ou le cérium (Ce), le restant étant formé de nickel (Ni) et d'impuretés occasionnelles.

2. Composition de superalliage selon la revendication 1, comptant 6,5 à 6,6 pour cent en poids de tantale.

3. Composition de superalliage selon la revendication 1, comptant 0 pour cent en poids de rhénium.

4. Composition de superalliage selon la revendication 1, comptant 0,5 pour cent en poids de rhénium.

5. Composition de superalliage selon la revendication 1 constituée, en pourcentage en poids, des éléments suivants : 6,3 d'aluminium (Al), 6,5 de tantale (Ta), 6,0 de chrome (Cr), 6,25 à 7,0 de tungstène (W), 2,0 de molybdène (Mo), 0,60 d'hafnium (Hf), 0,0 (Re), 7,5 de cobalt (Co), éventuellement, 0,03 à 0,6 de carbone (C), éventuellement, jusqu'à 0,004 de bore (B), éventuellement jusqu'à 0,03 au total d'un ou plusieurs éléments de terres rares choisis parmi l'yttrium (Y), le lanthane (La) ou le cérium (Ce), le restant étant formé de nickel et d'impuretés occasionnelles.

6. Article formé d'une composition de superalliage selon la revendication 1 ou la revendication 5.

7. Article selon la revendication 6, comprenant un composant de moteur de turbine à gaz.

8. Article selon la revendication 7, comprenant une tuyère ou un segment de tuyère de turbine à haute pression.
